

## UNITED STATES PATENT OFFICE.

WILLIAM M. BURTON, OF CHICAGO, ILLINOIS, ASSIGNOR TO STANDARD OIL COMPANY, OF CHICAGO, ILLINOIS, A CORPORATION OF INDIANA.

## FLUXING OIL.

No Drawing.

Application filed November 21, 1918. Serial No. 263,535.

*To all whom it may concern:*

Be it known that I, WILLIAM M. BURTON, a citizen of the United States, residing at Chicago, in the county of Cook and State 5 of Illinois, have invented a new and useful Improvement in Fluxing Oils, of which the following is a specification.

The present invention relates to the art of treating petroleum oils and will be fully 10 understood from the following specification.

It has been discovered that it is possible to produce from a petroleum base by the process which will hereinafter be described, a product which forms a perfect flux for all 15 commercially used asphalts, not only synthetic asphalts or asphalts produced from mineral oils but likewise natural asphalt such as Trinidad and Cuban asphalt.

The product used as a base for the preparation of the fluxing oil of the present invention is the tar or residue resulting from the operation of cracking petroleum hydrocarbons according to the method described in the patent to William M. Burton, No. 25 1,049,667, of January 7, 1913. As set forth in the said patent, a quantity of relatively heavy petroleum hydrocarbons, such as fuel oil or gas oil, having a boiling point of about 500° F. and upwards, is distilled under pressure, conditions being such that decomposition or cracking of the oil occurs and there is produced a distillate of the character of gasoline. Simultaneously with this cracking operation and the formation of the light 30 distillate referred to there is a change in the character of the oil body within the still. The distillation process is ordinarily interrupted when there still remains within the still a considerable residue which may in 35 some cases amount to as much as fifty per cent of the original charge. This residue, known as "pressure tar" is in accordance with the present invention now removed from the pressure still in which it was 40 formed and introduced into another still equipped with means for supplying open steam to the still contents.

The charge of pressure tar having been 45 introduced into this still is now subjected to distillation, the body of the still being fired in the usual manner and open steam

simultaneously blown through the oil body within the still. Samples of the contents of the still are taken from time to time and tested for specific gravity and viscosity. 55 When the specific gravity has reached about 1.06 (at 60° F.) the Engler viscosity will be about 6 (at 212° F.). The process is now at an end. The contents of the still are withdrawn and constitute the fluxing oil of 60 the present invention. As stated above, this oil is found to be a perfect flux, readily mixing in all proportions with both the natural and artificial asphalts known to the trade.

While in the foregoing there is described a specific process in accordance with the invention, together with the exact characteristics of the product produced thereby, it will be understood that this is by way of 70 illustration only and that the invention is not limited to the detailed specifications given, except in so far as these form a part of the accompanying claims, in which it is intended to claim all novelty inherent in the 75 invention as broadly as is permissible in view of the prior art.

What is claimed is:

1. A residue of petroleum distillation capable of fluxing natural and artificial asphalts and having an Engler viscosity at 212° F. of the order of 6 and a specific gravity of the order of 1.06 at 60° F.

2. The asphalt fluxing oil constituting a liquid residue having a specific gravity 85 slightly above that of water and having the characteristics of an oil derived from the tarry residue of the pressure cracking of a petroleum oil, said fluxing oil being free of lighter constituents.

3. The method of producing an asphalt fluxing oil which consists in distilling under pressure a petroleum product of the approximate character of fuel oil until a substantial proportion of said product has been converted into hydrocarbons of lower boiling point and distilled off, and subjecting the tarry residue of such pressure distillation to distillation in the presence of open steam until its Engler viscosity at 212° F. 95 is approximately 6.

WILLIAM M. BURTON.